

# UNITED STATES PATENT OFFICE.

DAVID REICHINSTEIN, OF ZURICH, SWITZERLAND.

## RUST-PREVENTING PROCESS.

1,395,730.

Specification of Letters Patent.

Patented Nov. 1, 1921.

No Drawing.

Application filed December 18, 1916. Serial No. 137,720.

To all whom it may concern:

Be it known that I, Dr. DAVID REICHINSTEIN, a citizen of the Republic of Switzerland, residing at Zurich, No. 51 Universitätsstrasse, Switzerland, have invented certain new and useful Improvements in Rust-Preventing Processes; and I do hereby declare the following to be a full, clear and exact description of the invention, such as will enable others skilled in the art to which it appertains to make and use the same.

It is well known that alkaline solutions, such as  $\text{NH}_4$ ,  $\text{NaOH}$ , act as rust preventers at room temperatures, because it is supposed that they produce an alkaline reaction having a retarding effect upon the formation of oxid. It is also known that iron surfaces can be provided with a rust-preventing coating of iron nitrid by heating the iron articles in a gaseous atmosphere capable of forming a nitrid. These processes are naturally not suitable for preventing the formation of rust on such iron surfaces, such as the parts of steam turbines, steam boilers, etc., which are exposed to the action of steam containing air at a high temperature. By the expression "iron surface" is meant here a surface composed exclusively of iron or only partly of iron, such as for instance a surface of nickel-steel or other iron alloys.

Contrary to the many existing theories of the formation of rust (see for instance Liebreich "Rost und Rostschutz" published by Vieweg & Sohn), the formation of rust can be completely explained if it is considered to be analogous to the dissolution of a metal in an acid solution containing an oxidizer (see article by Reichinstein in the *Zeitsch. für Elektrochemie* 1914 and 1915). According to this view the formation of rust may be represented by the following reactions.

1. Adsorption of the oxidizer for instance atmospheric oxygen by the iron surface.

2. Decomposition of the oxidizer in the adsorption volume of the iron surface, for instance,



3. Chemical reaction between the constituents of the adsorption volume:



4. Association of the  $\text{Fe} \cdots$ - and  $\text{OH} \cdots$ -ions, if their solubility product is exceeded:



All the reactions therefore take place in

the homogeneous phase of the iron surface (= adsorption volume). The  $\text{H} \cdots$ - and  $\text{OH} \cdots$ -ions pass into the adsorption volume from the adjacent liquid phase by prevention. If the iron is in contact with water vapor or steam, the latter is adsorbed partly by the iron surface and becomes dissociated therein:



The passive effect of the oxidizer consists in the increase of the  $\text{O}$ -concentration of the adsorption volume, so that according to the displacement principles (Reichinstein 1 c.) the  $\text{Fe}$ - and  $\text{H} \cdots$ -concentration is diminished, and this must necessarily lead to a retarding of the velocity of the reaction 3.

Analogously to that, the poisonous effect consists in the adsorption of poison by the iron surface which leads to the diminution of the concentrations of all the substances that share in the reaction 3.

The rust-preventing effect of alkalis consists in the fact that the reaction 3 is slow, and the reaction 4 is rapid, so that a diminution of the  $\text{H} \cdots$ -ions-concentration by the alkali has an appreciable effect upon the velocity of the formation of rust.

This has led the inventor further to the use of volatile bases, for instance ammonia, for the purpose of rust-prevention in cases where the iron is in contact with water vapor or steam containing air.

Experiments have shown that iron which is exposed to a mixture of air, water vapor and ammonia at  $100^\circ \text{C}$ , does not rust at all, whereas without ammonia, rusting begins after barely five minutes.

### Example.

Ammonia is added to the feed water of the steam boiler of a steam turbine. The ammonia passes with the steam into the turbine whereby the latter is protected from rust.

The ammonia can also be mixed in gaseous form under high pressure with the steam of the turbine by means of a special apparatus. Instead of using pure ammonia, the turbine may be blown through from time to time with a mixture of nitrogen and ammonia under high pressure. The volatile base may also be produced by introducing a salt of the respective base into the steam boiler, and adding by means of a special apparatus a less volatile base, for instance  $\text{NaOH}$ , drop by drop into the boiler. Other bases such as anilin, which are either volatile them-

selves or with steam, may be employed for the same purpose.

The process according to the present invention provides a rust-preventing agent in 5 gaseous form, so that the rust-preventing agent will come into contact even with the difficultly accessible parts of the surfaces that are to be protected.

In order to furnish an indication of the 10 quantity of ammonia it is desirable to employ, it may be stated that, in the case of a 3000 H. P. turbine built for a normal steam pressure of 165 lbs. per square inch and a speed of 3000 revolutions per minute, about 15 600 kgs. of steam is admitted to the turbine in fifteen minutes, and a solution of ammonia was injected at two points, namely, immediately behind the regulating slide valve, and at the top in front of the last slide 20 ring but two. The ammonia solution had a strength of  $\frac{1}{10}\%$ , and the admission took place as follows: during two minutes before the heating up of the turbine, during the heating up, and during the working from 25 12 noon to 6 p. m. every hour for one minute, then at 6 p. m. for five minutes, during the shutting down of the turbine. The total amount injected was about 40 liters (these 40 liters contain 80 grs. of  $\text{NH}_3$ ). 30 It is to be observed that when ammonia or ammonium salts are, in accordance with the present invention, added to boiler waters they are not added in conjunction with or-

ganic materials, graphite and such other substances as are considered to assist in the direction of preventing incrustation, thus when a less volatile base such as sodium-hydroxid is, in carrying the present invention into effect, added to the boiler water, it is added solely in the proportion necessary to set free 40 the more volatile as indicated above.

It is however to be remarked that from the above explanatory statement it is not to be inferred that the water may not have been treated by a recognized process.

What I claim is:

1. A process for preventing the rusting of iron surfaces of steam operated apparatus contacted by steam containing air at high temperatures, which comprises adding from 50 time to time a gaseous base mixed with nitrogen to the steam containing air.

2. A process for preventing the rusting of iron surfaces of steam-operated apparatus contacted by steam containing air, which 55 comprises blowing from time to time through such apparatus with the steam and air mixture ammonia and nitrogen under pressure.

In testimony that I claim the foregoing as my invention, I have signed my name in 60 presence of two subscribing witnesses.

DR. DAVID REICHINSTEIN.

Witnesses:

ARNOLD LEHNER,  
CARL GREBLEIN.